

Oct. 25, 1932.

W. B. PLUMMER

1,884,206

RECONDITIONING ALLOY STEEL

Filed July 18, 1930



Fig. 1



Fig. 2



Fig. 3

Inventor:

William B. Plummer

By Bruce K Brown Atty.

## UNITED STATES PATENT OFFICE

WILLIAM B. PLUMMER, OF CHICAGO, ILLINOIS, ASSIGNOR TO STANDARD OIL COMPANY (INDIANA), OF CHICAGO, ILLINOIS, A CORPORATION OF INDIANA

## RECONDITIONING ALLOY STEEL

Application filed July 18, 1930. Serial No. 469,001.

This invention relates to a process and apparatus for reconditioning alloy steel and it pertains more particularly to the temperature resistant steels used in petroleum refinery apparatus, such as hydrogenation units, cracking units, pipe stills, tubes, soaking drums, reaction chambers, etc.

The object of my invention is to minimize corrosion and prevent embrittlement of alloy steel used in petroleum refinery apparatus whereby replacement costs may be minimized and safety may be insured. A further object is to operate hydrogenation units, cracking units, pipe stills, etc. indefinitely with a minimum amount of shut-down time for repair and replacement. A further object is to recondition alloy steel, preferably in situ, and to provide furnace structure whereby this can be accomplished. Other objects will be apparent from the following detailed description.

I have discovered that if an alloy containing over .07% carbon is periodically heated to temperatures over about 1500° F., preferably of about 1750° F. (in the absence of additional carbon) its life will be lengthened indefinitely, corrosion will be minimized, and embrittlement and formation of weak spots will be prevented. I believe that this is accomplished by eliminating segregation of carbon and/or carbides at grain boundaries. The high temperatures apparently cause the carbon, which has slowly diffused from the grains, to be reabsorbed thereby so that there will be no weak spot due to accumulated carbon, chromium carbides or other inter-crystal accretions.

The heating of tubes, soaking drums, stills, etc., to temperatures of the order of 1750° F. requires material modifications to apparatus which is generally used in refineries. At these high temperatures the safe load is only a few hundred pounds per square inch and the tubes or other apparatus must be supported thoroughly and at frequent intervals against sagging during the period of heating. In order that uniform temperatures may be attained and maintained throughout the entire volume of the furnace, the heating must be uniform and it must be

initiated by slow fire; extra burners should be provided to insure proper heating of points farthest removed from the usual burners and the furnace gases should be tempered by the recirculation of large proportions of the products of combustion. If non-alloy tubes are used in parts of the stills or apparatus, these non-temperature resistant tubes must be protected against the high temperatures used, preferably by introducing cold gases through the furnace wall for forming a protecting shield around these tubes.

The walls of ordinary furnaces are not designed to withstand such temperatures and they must be modified accordingly, preferably by using fire brick throughout all sections wherein alloy tubes are used.

I prefer to utilize the heat in the exit gases during this high temperature heating period by means of suitable economizers, preheaters or exchangers; unless such means are employed it may be necessary to prevent excessive stack temperatures by introducing a large volume of air or inert gas directly into the top flue gases leaving the furnace.

The tubes, reaction chambers and other apparatus used in refining petroleum oils frequently become coated internally with deposits of coke (carbon). This coke should be removed before the apparatus is reconditioned by high heat treatment because at such high temperatures additional carbon may be dissolved by the alloy which in turn will increase the rate of carbon and/or carbide segregation thereafter. It is of importance that the carbon content of alloy be maintained at a low figure. If carbon or coke has deposited on tube walls it should be removed during the early stage of the high temperature treatment by passing air through the tubes until carbon dioxide no longer appears in the exit gas. Any means may be used, however, for removing the carbon from the apparatus prior to the reconditioning by heat treatment.

It is extremely important that the furnace structure be designed to withstand abnormal expansion and contraction due to the abnormal temperature changes. Tubes must not only be supported at more frequent intervals to prevent sagging, but they must also

be given more leeway for expansion. I prefer to use the so-called "up-shot" or DeFlorez type of heater wherein the tubes are vertically mounted in a circle around a central burner. Even this type of a still should 5 be especially built to withstand higher temperatures and greater expansion than that heretofore encountered.

The invention will be more clearly understood from the following detailed description of preferred embodiments and from the accompanying drawing wherein:

Figure 1 is a transverse vertical section through a pipe still taken along the lines 1—1 of Figure 2.

Figure 2 is a vertical section through the same pipe still taken along the lines 2—2 of Figure 1, and

Figure 3 is a vertical section through an up-shot furnace of the DeFlorez type.

The pipe still or furnace structure does not differ from ordinary pipe still or furnace structure except that provision is made for heating the alloy steel tubes to higher temperatures. In other words, additional burners may be required, additional tube supports may be used, steel tubes may be protected by the addition of cold gases, and furnace temperatures may be tempered with recycled flue gases. Parts of the furnace which are exposed to unusually high temperatures are designed to withstand the additional expansion incident thereto. Otherwise the structure is not materially different from conventional furnace structures and it will therefore not be described or shown in great detail.

Referring to Figure 1, pipe still 10 may consist of a steel frame lined with insulating material, the insulation of the upper part being preferably of fire brick. Heater tubes 11 are suspended from a roof by tube supports 12 and since these tubes are to be exposed to extremely high temperatures the tube supports are spaced close enough together to prevent tubes from sagging between supports. The ends of the tubes are accessible from openings 13 in the pipe still wall and when the return bends 14 are removed therefrom carbon may be removed by scraping or by other conventional methods. Ordinarily the furnace is heated by burner 15, but to obtain the unusually high temperatures hereinafter described, I provide additional burners 16, particularly for heating remote parts of the alloy 55 tubes. In order to temper the gases in the furnace, I may recycle flue gas from the flue 17 through pipe 18, compressor 19 and pipe 20 back to the combustion chamber. A baffle wall 21 separates the combustion chamber 60 from the convection chamber and in order to protect steel tubes 21 in the convection chamber I may introduce cold gas through pipe 22.

Referring to Figure 3, the furnace 23 is a 65 steel cylinder lined with insulating material

24. Outer pipes and inner pipes 25 and 26 respectively are spaced at intervals around the circumference of the cylinder and extend through the top and the bottom thereof. These pipes are connected by return bends 70 27 so that they form a continuous conduit; they may be cleaned at intervals by removing the return bends 27 therefrom and inserting cleaning tools therein.

Pipes 25 and 26 are heated by the usual 75 burner 28, but in practicing my invention I use additional burners 29 to heat those portions of the tubes which are remote from the usual burner. I may temper the gases in the furnace by cycling flue gas through pipe 80 30, compressor 31 and pipe 32. In order to protect the steel tubes 33 in economizer section 34 I may introduce cold gases through pipe 35.

My invention may be applied to any high 85 temperature alloy steel and as a specific example I may use a steel containing 18% chromium, 8% nickel, .15% carbon, small proportions of the usual impurities, etc., and the balance iron. This alloy is particularly 90 well suited for withstanding high internal pressures and for resisting shock at elevated temperatures. If the tubes are used in a hydrogenation heater they may be operated at about 850° F. under a pressure of about 95 150-300 atmospheres. At frequent intervals it may be necessary to clean the apparatus and to remove deposited carbon. At such times (when tests or experience indicate that the steel has deteriorated) after the carbon 100 has been removed I may slowly fire the furnace and raise the temperature of the tubes 105 to about 1750° F., using auxiliary burners, recirculated hot gases, etc. for attaining and maintaining a uniform high temperature. The time required for the reconditioning varies with the temperature employed; at 1750° F. it is about 36 hours. At 1500° F. the time required is probably 45 or 50 hours, and higher temperatures will require less 110 time.

At these high temperatures it appears that the carbon which is diffused from the crystals and which has segregated between the crystals is re-dissolved so that a tenacious bond is 115 once more obtained between these crystals. While I believe that this is the explanation of my improved results I do not limit myself to any theory. Furthermore, I do not limit myself to the precise temperatures or other details hereinabove set forth except as defined by the following claims.

The term "carbon" in the following claims includes carbon in the combined state as well as elemental carbon.

I claim:

1. In the refining of petroleum oils, the method of reconditioning deteriorated alloy steel oil-heating tubes which comprises cleaning the surface of the tubes to remove de- 130

5 posited carbon, heating the tubes in situ to a temperature of over 1500° F. and maintaining the tubes at the elevated temperature for a sufficient period of time to restore the non-brittle condition of the tubes.

6 2. The process of claim 1 wherein the period of time is more than thirty-six hours.

10 3. In the refining of petroleum oils, the method of reconditioning deteriorated oil-heating tubes composed of alloys containing more than 6% nickel, more than 15% chromium, and more than 0.07% carbon which comprises cleaning the surfaces of the tubes to remove deposited carbon, heating the tubes in situ to a temperature of over 1500° F. and maintaining the tubes at the elevated temperature for a sufficient period of time to restore the non-brittle condition of the tubes.

15 4. The combination of claim 3 wherein the period of time is more than thirty-six hours.

20 Signed this 14th day of July, 1930, at Chicago, in the county of Cook, State of Illinois.

WILLIAM B. PLUMMER.

35

40

45

50

55

60